

# UNITED STATES PATENT OFFICE.

BENJAMIN A. PEACOCK, OF PHILADELPHIA, PENNSYLVANIA, ASSIGNOR TO HASLUP & PEACOCK, INC., OF NEW YORK, N. Y., A CORPORATION OF NEW YORK.

## PROCESS OF OBTAINING POTASSIUM SULFATE.

1,279,145.

Specification of Letters Patent. Patented Sept. 17, 1918.

No Drawing.

Application filed February 8, 1918. Serial No. 216,078.

*To all whom it may concern:*

Be it known that I, BENJAMIN A. PEACOCK, a citizen of the United States, residing at Philadelphia, in the county of Philadelphia and State of Pennsylvania, have invented certain new and useful Improvements in Processes of Obtaining Potassium Sulfate; and I do hereby declare the following to be a full, clear, and exact description 10 of the invention, such as will enable others skilled in the art to which it appertains to make and use the same.

This invention relates to a process of extracting combined potassium from hydrous silicate minerals containing the same, such as glauconite, sericite, muscovite, etc., and has for its object to improve and lessen the costs of the methods heretofore proposed.

With these and other objects in view the invention consists in the novel steps and combinations of steps constituting the process, as will be more fully hereinafter disclosed and particularly pointed out in the claims.

In order that the invention may be clearly understood it is said:—It has been heretofore proposed to treat minerals of the kind above mentioned with boiling acids, such as sulfuric, for example, but as said minerals usually contain relatively large proportions of aluminum oxide, and also may contain iron oxides, which combine with the acid employed to extract the combined potassium, it is found that a very large percentage of said acid is expended in producing sulfates of aluminum and iron, which have very little commercial value, and that therefore the cost of the potassium sulfate produced is very greatly increased. These facts may be illustrated by an example. A ton of ordinary run of the mine glauconite will contain acid consuming oxides and will require acid as follows:—

|    |                           |                       |                  |
|----|---------------------------|-----------------------|------------------|
| 45 | Ferric oxid, 295 lbs,     | 60° B. sulfuric acid. | 700 pounds acid. |
|    | combines with             |                       |                  |
|    | Ferrous oxid, 95 lbs,     |                       | 167 pounds acid. |
|    | combines with             |                       |                  |
|    | Alumina, 175 lbs., com-   |                       | 649 pounds acid. |
| 50 | bines with                |                       |                  |
|    | Potassium oxid, 125 lbs., |                       | 168 pounds acid. |
|    | combines with             |                       |                  |

Total acid required— 1,684 pounds acid.

55 Of the total acid, 1,684 pounds, required to decompose a ton of glauconite it will thus

be seen that only 168 pounds, or say 10% is utilized in producing the desired potassium sulfate, the remaining 90% of acid is thus practically lost in producing products 60 of little or no commercial value.

I have discovered, on the other hand, that if the comparatively inexpensive sulfates of aluminum and iron, ferric and ferrous, be mixed in the first instance with a naturally occurring hydrous potassium bearing mineral such as glauconite, and in such quantities as to supply only slightly more sulfuric anhydrid than is necessary to form a sulfate with all the potassium present, and 70 if the mixture be heated well above say 100° C., for some hours, say twenty-four or forty-eight, or less, according to the temperature employed, the mineral is decomposed to the extent that the potassium present is converted into a sulfate and may be extracted with water. That is to say, if only aluminum oxids are present in the mineral I mix with the latter aluminum sulfate, but if both aluminum and iron oxids 80 are present in the mineral, I add the sulfates of both aluminum and iron.

I have further found that the sulfates of iron and aluminum need not be added to the mineral, but may be formed therein and 85 then decomposed. That is to say, by restricting the amount of acid required to that slightly in excess of what is necessary to convert all the potassium present into a sulfate, I find that equivalent amounts of 90 iron and aluminum sulfates will be first formed with very little if any potassium sulfate. Later upon raising the temperature well above 100° C., to say 200° C., or 250° C., 95 these said sulfates are decomposed with the formation of potassium sulfate which is then leached out with water.

Of course, the mineral is preferably employed in a finely divided condition, or ground to say 60 mesh, and impure or relatively cheap acids are preferred to lessen the costs of the process.

It is obvious that those skilled in the art may vary the details of the process without departing from the spirit of the invention, and therefore, I do not wish to be limited to the above disclosure except as may be required by the claims.

What I claim is:—

1. The process of extracting combined 110 potassium from a hydrous mineral containing the same, such as glauconite, which con-

sists in providing a mixture containing said mineral and aluminum sulfate, the latter being present in a quantity only slightly in excess of that required to supply sufficient sulfuric anhydrid to combine with all the potassium present; heating said mixture to a temperature sufficient to decompose said sulfate in the presence of said potassium to form potassium sulfate; and extracting the latter from the mass, substantially as described.

2. The process of extracting potassium sulfate from glauconite which consists in providing a finely divided mixture containing glauconite and aluminum sulfate, the

latter being present in a quantity only slightly in excess of that required to supply sufficient sulfuric anhydrid to combine with all the potassium present; heating said mixture to a temperature above 100° C. for a time sufficient to form the desired potassium sulfate; and extracting the latter with water, substantially as described. 20

In testimony whereof I affix my signature in presence of two witnesses.

BENJAMIN A. PEACOCK.

Witnesses:

OWEN CRAVEN,

W. M. E. BLAIR.

Copies of this patent may be obtained for five cents each, by addressing the "Commissioner of Patents, Washington, D. C."